

Patented Feb. 12, 1924.

1,483,519

# UNITED STATES PATENT OFFICE.

ROBERT A. PHAIR, OF ALLENDALE, NEW JERSEY, ASSIGNOR, BY MESNE ASSIGNMENTS, TO H. KOHNSTAMM & CO., INC., A CORPORATION OF NEW YORK.

## SOURING COMPOSITION AND METHOD.

No Drawing. Original application filed July 18, 1921, Serial No. 485,642. Divided and this application filed June 15, 1922. Serial No. 568,650.

To all whom it may concern:

Be it known that I, ROBERT A. PHAIR, a citizen of the United States, residing in Alendale, New Jersey, have invented certain new and useful Improvements in Souring Compositions and Methods, of which the following is a specification.

In my application No. 485,642, filed July 18, 1921, I have described certain improvements in the materials and steps used in laundry work and in the analogous treatment of textile materials. The present application is a division thereof, directed particularly to the materials and steps used in souring operations. After the usual laundering operations it is customary to bleach the goods and then to rinse them so as to remove the bleaching material. But there is generally a residue of the bleaching material and certain products of the bleaching operation, which cannot be removed by rinsing, and the goods should be treated to a subsequent souring operation. My invention contemplates an improvement on such souring operations by adding to the usual laundry sour or to any suitable laundry sour a chlorine-neutralizing agent.

The laundry sour which I propose using comprises a compound of fluorine having an acid reaction in combination with a reducing agent or other material adapted to neutralize the destructive effect of chlorine, hypochlorous acid and other products of the acid decomposition of hypochlorites from the bleach which was used in a previous stage. One example of such an improved sour is a mixture of sodium acid fluoride and sodium sulfite; another is sodium silicofluoride and sodium bisulfite.

The advantages which this sour possesses over others previously used are several. Even if it is not thoroughly rinsed out in the next operation, it is not destructive of the goods. The decomposition products of the hypochlorites used in the bleaching operation have an intense destructive action, and such products are entirely removed or neutralized by this sour. Any of the bleach in more or less loose combination with stains in the fabric, and which would ordinarily cause holes therein in time, is neutralized. Thus the color of print goods for example, and also the fabric are saved from such de-

structive effects. Also any alkali which is present either free or in combination with the oxycelluloses is neutralized and the goods are thereby whitened. Certain stains are removed by reduction and decolorizing of them. Any insoluble lime magnesia soaps which may remain on or in the goods are so modified as to be rendered soluble in alkaline solution. By this souring operation the goods are put in the best shape for the bluing operation which follows and which is succeeded by the final rinsing in clear water.

In the treatment of textile materials, and particularly vegetable fibers, to remove the fats, waxes and other dirt prior to bleaching, mercerizing or dyeing, a sour of the same character is found very advantageous; that is, a sour composed of an acid compound of fluorine with a reducing agent as above described. The acid compound of fluorine combines with any alkali present, to remove stains and whiten the material and also to remove any lime salts caused by the water or by the materials used. Sulphuric and hydrochloric acids have been largely used for this purpose, but any traces thereof left in the goods will rot the latter, whereas the acid compounds of fluorine will not do so. Also a very much smaller quantity of the latter may be used because of the comparative sluggishness of sulphuric and hydrochloric acids; in fact about one-fifteenth as much of the acid compound of fluorine will do the same amount of work. This use of an acid compound of fluorine in the treatment of textile materials after boiling out of the unbleached vegetable fibers is believed to be new, either alone or in combination with the reducing agent.

Though I have described with great particularity of detail certain embodiments of my invention, yet it is not to be understood therefrom that the invention is restricted to the particular steps and materials described. Various modifications thereof may be made by those skilled in the art without departing from the invention as defined in the following claims.

What I claim is—

1. In laundering or treating textile materials the method which consists in subjecting the goods after the bleaching, to

- treatment with a composition which sours and neutralizes the destructive effect of the bleach.
2. In the laundering or treating of textile materials the method which consists in subjecting the goods to a sour after bleaching, said sour containing an acid compound of fluorine and an agent adapted to neutralize the destructive effect of the bleach.
- 10 3. In the laundering or treating of textile materials the method which consists in subjecting the goods to a sour containing an acid compound of fluorine with a reducing agent.
- 15 4. In the treating of textile materials to remove fats, waxes or other dirt, the method which includes boiling out the fibers and then subjecting the material to a sour containing an acid compound of fluorine.
5. A souring composition for treating 20 textile materials comprising an acid compound of fluorine and a neutralizing agent opposed to the destructive action of bleaches.
6. A souring composition for treating textile materials after bleaching comprising an 25 acid compound of fluorine and a reducing agent.
7. A souring composition for treating textile materials including a chlorine-neutralizing agent. 30

In witness whereof, I have hereunto signed my name.

ROBERT A. PHAIR.